

No. 633,671.

Patented Sept. 26, 1899.

Z. VALDEZ.

TOY TORPEDO.

(Application filed Feb. 7, 1899.)

(No Model.)



Witnesses

M. M. Ginnis

J. C. des Granges.

Inventor

Zefirino Valdez

By Hazard & Marpham  
Attorneys

# UNITED STATES PATENT OFFICE.

ZEFERINO VALDEZ, OF LOS ANGELES, CALIFORNIA.

## TOY TORPEDO.

SPECIFICATION forming part of Letters Patent No. 633,671, dated September 26, 1899.

Application filed February 7, 1899. Serial No. 704,805. (No model.)

*To all whom it may concern:*

Be it known that I, ZEFERINO VALDEZ, a citizen of the United States, residing in the city of Los Angeles, county of Los Angeles, 5 State of California, have invented a new and useful Toy Torpedo, of which the following is a specification.

My invention relates to that class of toy torpedoes which are designed to be thrown 10 against a hard substance and thereby produce detonation; and the objects of my invention are, first, to produce a toy that will amuse children; second, to provide a torpedo that will not only produce detonation, but 15 will also give out luminosity as it rolls along and may give out a succession of detonations from one torpedo. I attain these objects by the torpedo described herein and illustrated in the accompanying drawing, which is a central section of my torpedo.

In the drawing, A represents a clay ball; B, a preservative coating; C, a fulminating compound.

Clay is molded into small balls, which are 25 thoroughly dried without artificial heat, as such heat has a tendency to make the clay too brittle and to cause holes therein. If the clay is brittle, the balls are too easily broken, and if full of holes they absorb too much of the 30 compound with which they are coated. After the balls are dry they are dipped in a preservative mixture B, composed of shellac and alcohol in the following proportions: one-fourth pound of gum-shellac to one pint of 35 alcohol. This is done to prevent the moisture remaining in the clay (it being impossible to dry it all out without too great a loss of time) from injuriously affecting the fulminating compound. This coating is then allowed 40 to dry on the balls. They are then dipped in a fulminating compound C, made as follows: One pound of gum-arabic is first thoroughly dissolved in one pound of water. In this mixture one pound of phosphorus is dissolved by a 45 steam-bath and the mixture is allowed to cool. When cool, one and one-fourth pounds of powdered chlorate of potash is thoroughly stirred into the mixture, which completes the fulminating compound.

The balls prepared as above are thoroughly coated with the fulminating compound and are placed in dry sand, in which they are

rolled, and then taken out and permitted to dry. When dry, they are again coated with the preservative compound and allowed to 55 dry, when they are ready for use.

If the torpedoes are manufactured for immediate use, the use of the preservative compound may be omitted, as it is only necessary to use it when it is desired to keep the torpe- 60 does some considerable length of time.

The torpedo is used as follows: It is thrown against any hard substance with some force and on striking will detonate that portion of the fulminating compound at the point of contact and will ignite the remainder, which will burn slowly as the ball rolls along. Should the ball strike another hard substance and the point of contact be covered with the fulminating compound, another explosion will 65 occur, and this will be repeated until all the fulminating compound is burned off the ball. It can also be used by gripping it tightly with the index-finger of one hand and then quickly forcing it out with the index-finger of the 70 other hand in any desired direction. The friction occasioned thereby will cause the ignition of the fulminating compound on the ball, which will burn as the ball flies through the air and give out a light like that of a dis- 75 charged Roman-candle ball.

Having described my invention, what I claim is—

1. A toy torpedo composed of a central ball of clay surrounded by a coating of fulminat- 85 ing compound composed of the following ingre- dients, viz: gum-arabic four parts; phosphorus four parts; and chlorate of potash five parts.

2. The herein-described toy torpedo, com- 90 prising a ball of dried clay forming the center thereof, a coating of gum - shellac sur- rounding said ball of clay, a coating composed of gum-arabic four parts, phosphorus four parts, and chlorate of potash five parts sur- 95 rounding the coating of shellac, and a coat- ing of shellac on the outside thereof.

In witness that I claim the foregoing I have hereunto subscribed my name, this 31st day of January, 1899, at Los Angeles, California. 100

ZEFERINO VALDEZ.

Witnesses:

G. E. HARPHAM,  
W. M. CASWELL.